# EUROPEAN PATENT APPLICATION

(11) **EP 4 484 585 A1**
(43) Date of publication of application: **01.01.2025**
(21) Application number: 23803620.6
(22) Date of filing: 11.05.2023
(51) Int. Cl.: C21D 8/02, C22C 38/00, C22C 38/14, C22C 38/58

(54) **STEEL SHEET AND METHOD FOR MANUFACTURING SAME**

(30) Priority: 12.05.2022 JP 2022079060
(71) Applicant: JFE Steel Corporation, Tokyo 100-0011 (JP)
(72) Inventor: OKUTANI, Masaomi, Tokyo 100-0011 (JP); TERAZAWA, Yusuke, Tokyo 100-0011 (JP); OHTSUBO, Hirofumi, Tokyo 100-0011 (JP)
(74) Representative: Haseltine Lake Kempner LLP
(86) International application number: PCT/JP2023/017811
(87) International publication number: WO 2023/219146

(57) **Abstract**

Provided is a steel plate having high strength and excellent multilayer-fill-welded joint CTOD properties even when thickness exceeds 100 mm. The steel plate has a defined chemical composition, and in a mid-thickness part, average effective crystal grain size is 20 µm or less and maximum effective crystal grain size is 150 µm or less, and at a 1/2 thickness position, composite inclusions containing sulfides containing Ca and Mn and oxides containing Al and having a circle equivalent diameter of 0.1 µm or more are present at a number density of 25/mm² to 250/mm².

## Description

### TECHNICAL FIELD

The present disclosure relates to steel material suitable for steel structures such as ships, marine structures, pressure vessels, line pipes, and offshore wind power generators. Specifically, the present disclosure relates to a thick, high tensile strength steel plate having a thickness exceeding 100 mm, that not only has excellent base metal strength and toughness but also has excellent joint CTOD properties in multilayer-fill-welded portions, and a method of producing same.

### BACKGROUND

In recent years, steel structures such as ships, marine structure, pressure vessels, line pipes, and offshore wind power generators are becoming larger. With such larger sizes, there is an increasing demand for higher-strength, thicker steel material for use as base metal.

In particular, when producing a steel plate having a thickness exceeding 100 mm, a mid-thickness part tends to have a decreased cooling rate and coarser crystal grains because of the increased thickness. Therefore, crystal grain refinement of the mid-thickness part is important to produce a steel plate where the mid-thickness part has excellent strength and toughness.

For example, in Patent Literature (PTL) 1, a technique is proposed to improve toughness of base metal by controlling rolling conditions to refine average effective crystal grain size of mid-thickness microstructure.

Conventionally, the Charpy test has been the main method for evaluating steel toughness. In recent years, a crack tip opening displacement test (hereinafter also referred to as CTOD test) has been increasingly applied to evaluate steel plates used in steel structures as a method to evaluate fracture resistance with higher precision.

The CTOD test evaluates resistance to occurrence of brittle cracks by introducing a fatigue precrack into a test piece at the location to be evaluated for toughness, subjecting the test piece to three-point bending, and measuring the amount of crack opening (plastic deformation) immediately before fracture.

Further, when steel plates are applied to steel structures such as ships, marine structures, pressure vessels, line pipes, offshore wind power generators, and the like, multilayer fill welding is used.

The heat-affected zone (hereinafter also referred to as "HAZ") of a multilayer fill weld is subjected to a plurality of different thermal cycles from each of the welding passes, forming a mixture of various microstructures. In particular, the HAZ in the vicinity of the weld line (coarse grain heat-affected zone: CGHAZ), coarsened by a preceding welding pass, is reheated into a two phase region of ferrite and austenite by a subsequent welding pass, and HAZ microstructure with martensite austenite constituent (MA) mixed in a coarse matrix (hereinafter also referred to as inter-critically reheated coarse grain heat-affected zone: ICCGHAZ) has particularly low toughness. Further, when crystal grain size of base metal microstructure is coarse, toughness of sub-critically reheated HAZ (SCHAZ) may become a problem.

According to the joint CTOD test method specified in British Standard (BS) EN10225-4 (2019) and American Petroleum Institute (API) Recommended Practice RP-2Z (2005), joint CTOD properties are required for the CGHAZ in the vicinity of the weld line and the SC/inter-critically reheated HAZ (SC/ICHAZ) boundary, which is the boundary of untransformed/transformed zones of the base metal during welding.

CTOD testing of welded joints is basically performed at full thickness, and therefore when the CGHAZ is the subject of evaluation, the region where a fatigue precrack is introduced includes the ICCGHAZ microstructure. That is, joint CTOD properties obtained by a joint CTOD test depend on toughness of the most brittle microstructure in the evaluation region, and therefore joint CTOD properties of the CGHAZ reflect the toughness of ICCGHAZ microstructure as well as CGHAZ microstructure.

Therefore, to improve joint CTOD properties at the CGHAZ, it is also necessary to improve toughness of the ICCGHAZ microstructure.

The HAZ microstructures described above are CGHAZ, ICHAZ, and SCHAZ in order of proximity from the weld line in the microstructure formed in one welding pass during multilayer fill (multi-pass) welding. ICCGHAZ is microstructure formed in multilayer fill welding when the CGHAZ is heated to a two phase region of ferrite and austenite by the thermal hysteresis of subsequent passes, and the location and frequency at which ICCGHAZ microstructure is formed can vary depending on how welding passes are layered.

Conventional toughness improvement techniques for the heat-affected zone (HAZ) have been suppression of austenite grain coarsening in the CGHAZ by fine particle distribution of TiN and the use of TiN as a ferrite nucleation site. However, in a bonded portion, TiN may be heated to a temperature range where TiN dissolves, and when low-temperature toughness requirements for a welded portion are stringent, satisfying the requirements mentioned above becomes difficult with only the effects mentioned above.

Further, techniques have also been used to suppress austenite grain growth by adding rare earth metal (REM) and dispersing REM acid sulfides formed, and making use of the ferrite nucleation ability of BN.

For example, PTL 2 describes a technique to suppress austenite grain growth and improve toughness of welded portions by adding REM in combination with Ti and dispersing the fine particles in steel.

Further, in PTL 3, a technique is proposed using boron nitride (BN) as a ferrite nucleation site in the heat-affected zone of large-heat input welding to refine HAZ microstructure and improve HAZ toughness.

Further, in PTL 4, as a measure for countering toughness decrease at the ICCGHAZ, a technique is proposed to increase base metal strength by adding Cu in addition to suppressing the formation of MA by decreasing C and Si content.

As described above, an increase in the amount of alloying elements is necessary to achieve both thicker and stronger steel plates, but the addition of large amounts of alloying elements leads to degradation of toughness of the multilayer-fill-welded HAZ, making securing desired low temperature joint CTOD properties more difficult.

To address this problem, PTL 5 describes a technique to improve low-temperature toughness by controlling hardness of a central segregation area.

### CITATION LIST

### Patent Literature

PTL 1: JP 6477993 B1
PTL 2: JP S60-184663 A
PTL 3: JP S61-253344 A
PTL 4: JP H05-186823 A
PTL 5: JP 5846311 B2

### SUMMARY

### (Technical Problem)

Here, the CTOD specification temperature in standards that specify joint CTOD properties (for example, API standard RP-2Z) is typically -10 °C.

However, to secure new resources in response to growing energy demand in recent years, the construction range of marine structures and the like has shifted to cold regions and deep-sea regions where resource development has not previously been possible. As a result, there is increasing demand for steel plates that are high-strength, thick, and capable of meeting CTOD specification temperatures that are even lower than those specified by the API standard.

According to investigation by the inventors, the conventional techniques described in PTL 1 to PTL 5 are unable to fully satisfy joint CTOD properties required for multilayer-fill-welded joints for low-temperature specifications in steel plates having a thickness exceeding 100 mm.

For example, although PTL 1 proposes rolling condition control for average effective crystal grain size refinement of mid-thickness microstructure, the technique has not been applied to steel plates having a thickness exceeding 100 mm. Further, to improve toughness in the mid-thickness part, refinement of average effective crystal grain size is insufficient; maximum effective crystal grain size also needs to be refined.

The technique proposed in PTL 2 to suppress coarsening of the austenite structure of the HAZ by adding REM in combination with Ti and dispersing fine particles in steel is targeted at steel material that has relatively low strength and low alloying element content. Therefore, the technique is not applicable to higher strength steel material with higher alloying element content, because the HAZ microstructure does not contain ferrite.

The technique proposed in PTL 3 is effective when HAZ microstructure is mainly composed of ferrite and a cooling rate of the heat-affected zone is slow, as in large-heat input welding. However, in multilayer fill welding, the heat input is relatively small, and further, the alloy component in the base metal is relatively large for steel plates exceeding 100 mm thickness. Therefore, in multilayer fill welding of steel plates, the HAZ microstructure becomes mainly bainite, and the HAZ toughness improvement effect described above cannot be obtained.

According to the technique proposed in PTL 4, satisfactory CTOD properties can be obtained at normal specification temperatures (-10 °C). However, the joint CTOD properties at lower temperature specification temperatures as mentioned above have not been investigated, and it may be considered that low-temperature CTOD specifications cannot be satisfied by only improving ICCGHAZ toughness through decreasing the base metal alloy component of C and Si.

Further, decreasing the alloying element content of base metal to improve the toughness of the ICCGHAZ is a technique that conflicts with securing strength for greater thickness, and may be considered difficult to apply to steel plates used in marine structures and the like.

PTL 5 proposes a technique for satisfactory joint CTOD properties at normal specification temperature (-10 °C) in steel plates having a thickness of 100 mm or less. However, for ultra-thick steel plates having a thickness exceeding 100 mm, mechanical properties equivalent to those of steel plates having thicknesses of 100 mm or less have not yet been obtained, and joint CTOD properties at even lower specification temperatures, as mentioned above, have not been investigated. Further, CTOD properties of the SC/ICHAZ boundary have also not been investigated.

Accordingly, in steel plates having a thickness exceeding 100 mm that combine high strength and low-temperature toughness, it is hard to say that a technology to improve the toughness of the CGHAZ, ICCGHAZ, and SCHAZ at the multilayer-fill-welded heat-affected zone has been established, and improving joint CTOD properties has been difficult.

The present disclosure is made in view of the problems described above faced by conventional technologies, and it would be helpful to provide a steel plate having a thickness exceeding 100 mm, high strength, excellent base metal toughness at low temperature, and excellent multilayer-fill-welded joint CTOD properties, as well as a method of producing same.

Hereinafter, high strength is defined as a yield stress of 325 MPa or more in the mid-thickness part in a tensile test. Excellent base metal toughness at low temperature is defined as having an absorbed energy of 100 J or more in the Charpy test at -40 °C in the mid-thickness part. Excellent multilayer-fill-welded joint CTOD properties is defined as a crack opening displacement of 0.4 mm or more at notch location CGHAZ and at the SC/ICHAZ boundary, respectively, at a test temperature of -20 °C.

### (Solution to Problem)

In order to solve the above problems, the inventors have extensively studied methods to improve CTOD properties in steel plates having a thickness exceeding 100 mm, while also achieving both high strength and improved low-temperature toughness of base metal. As a result, the inventors made the following discoveries.

Strength and toughness are strongly correlated with crystal grain size, and therefore in order to achieve both high strength at the mid-thickness part and low-temperature toughness in steel plates having a thickness exceeding 100 mm, crystal grain refinement in such regions is essential. When refining crystal grains, refining average effective crystal grain size is also important, but when coarse crystal grains are mixed even partially among such fine crystal grains, the coarse crystal grains become the weakest part of the crystal grains and become fracture origins. That is, material properties are governed not only by the average grain size, but also by the maximum grain size. Therefore, not only crystal grain refinement but also homogenization is essential.

With regard to the above, the inventors have found that the desired strength and toughness can be secured by making the maximum effective crystal grain size to 150 µm or less while keeping the average effective crystal grain size to 20 µm or less, in the base metal microstructure in the mid-thickness part, as described below.

However, with conventional technology, in a steel plate having a thickness exceeding 100 mm, it is difficult for strain to enter the mid-thickness part during rolling, and difficult to refine the average effective crystal grain size of base metal microstructure of the mid-thickness part to 20 µm or less.

Further, even when strain is appropriately introduced into the mid-thickness part and the average effective crystal grain size can be refined, then when coarse grains are mixed in, the coarse grains still become fracture origins.

The inventors discovered that such problems can be solved by eliminating coarse crystal grains that have a maximum effective crystal grain size exceeding 150 µm.

However, with conventional technology, eliminating coarse crystal grain that have a maximum effective crystal grain size exceeding 150 µm is difficult, particularly in steel plates having a thickness of 100 mm or more.

As a result of the extensive studies, the inventors discovered that these problems can be solved by the following methods.
(1) When mid-thickness temperature is in a temperature range of T₁ °C or more, which is a recrystallization temperature range, rolling with an average rolling reduction per pass (average of the rolling reduction in each pass) of 3 % or more and a cumulative rolling reduction ratio (cumulative rolling reduction/rolling start thickness) of 25 % or more can introduce sufficient strain to the mid-thickness part, which results in recrystallization to refine and homogenize crystal grains. Next, after avoiding rolling in a partial recrystallization temperature range (T₁ °C to T₂ °C) where recrystallized grains and coarse recovered grains are generated, rolling is performed at T₂ °C or less, which is a non-recrystallization temperature range, with a cumulative rolling reduction ratio of 30 % or more. According to these rolling operations, even in steel plates having a thickness exceeding 100 mm, average effective crystal grain size can be made 20 µm or less while also making the maximum effective crystal grain size 150 µm or less in the mid-thickness part.

Accordingly, in steel plates having a thickness exceeding 100 mm, in addition to clearly defining the recrystallization temperature range of T₁ °C or more and the non-recrystallization temperature range of T₂ °C or less and avoiding rolling at the partial recrystallization temperature (T₁ °C to T₂ °C), where recrystallization grains and coarse recovered grains are generated, desired fine and uniformly-sized grain microstructure can be obtained in the mid-thickness part by rolling under the conditions described above at temperatures of T₁ °C or more and T₂ °C or less.

Hereinafter, the mid-thickness part is a region from the center in the thickness direction (1/2 position) to a thickness of 10 % of the steel plate toward both main surfaces of the steel plate.

(2) When Ca, O, and S content in steel is controlled within the range of 0 to 1.5 in atomic concentration ratio (ACR) indicated in the following expression, inclusions become composite inclusions containing Ca sulfides partially containing Mn in solid solution and Al oxides. $ACR = \left\{\left[Ca\right]-\left(0.18+130 \left[Ca\right]\right)\times \left[O\right]\right\} / 1.25 / \left[S\right]$

Adding large amounts of alloying elements is essential when producing high strength, thick steel plates, and therefore it has conventionally been difficult to secure sufficient joint CTOD properties at low temperatures for a multilayer-fill-welded HAZ.

As a result of the extensive studies, the inventors discovered that by using composite inclusions containing two types of inclusion, that is, sulfides containing Ca and Mn and oxides containing Al, the composite inclusions can exist stably even in a region in the vicinity of the weld line where the temperature is increased to a high temperature, and the effect of suppressing austenite grain coarsening can be fully exhibited. Further, the inventors discovered that a Mn-poor layer is formed around the composite inclusions, which has a nucleation effect (nucleation site effect) on bainite and the like.

That is, when the complex inclusion having a nucleation effect is present in austenite grains, nucleation occurs not only from austenite grain boundaries but also from within the austenite grains, resulting in a finer finally obtained HAZ microstructure. As a result, HAZ toughness and joint CTOD properties are improved.

Further, the inventors discovered that the size of such composite inclusions needs to be 0.1 µm or larger in circle equivalent diameter in order to fully exhibit the nucleation site effect due to the composite inclusions described above.

Further, at least one composite inclusion needs to be present in the austenite grains of the HAZ when weld temperature is increasing in order to fully utilize refinement of the HAZ microstructure due to the nucleation site effect. In particular, austenite grain size in the vicinity of the weld line reaches about 200 µm or more, and therefore the inventors discovered that the number density of composite inclusions need to be 25/mm² or more in order for the finally obtained HAZ microstructure to be sufficiently fine. On the other hand, toughness of the composite inclusions themselves is low, and therefore the presence of an excessive amount of composite inclusions can instead reduce the HAZ toughness. In particular, the number of composite inclusions needs to be appropriately controlled in the mid-thickness part, where element segregation exists and multilayer-fill-welded HAZ toughness is poor. The inventors discovered that good multilayer-fill-welded joint CTOD properties are obtainable by making the number density of the composite inclusions 250/mm² or less.

(3) Generally, in an element segregation region of the mid-thickness part of a slab, alloying elements are concentrated and thus coarse inclusions are dispersed at low density.

As a result of the extensive studies, the inventors discovered that rolling at a high mid-thickness temperature of T₁ °C or more, with an average rolling reduction per pass of 3 % or more and a cumulative rolling reduction ratio of 25 % or more, can increase the strain applied to the mid-thickness part, elongate and break up coarse inclusions, and distribute fine inclusions to a high density. Further, the inventors discovered that such inclusions can help secure the HAZ toughness improvement effect.

(4) It is known that the toughness of base metal governs joint CTOD properties at the SC/ICHAZ boundary. As a result of the extensive studies, the inventors discovered that in order to satisfy joint CTOD properties at the SC/ICHAZ boundary at a test temperature of -20 °C, improving base metal toughness by crystal grain refinement and homogenization is required, such that the maximum effective crystal grain size is 150 µm or less and the average effective crystal grain size is 20 µm or less in the base metal microstructure.

Normally, in steel plates having a thickness exceeding 100 mm, the cooling rate of the mid-thickness part is smaller and crystal grains become coarser. Therefore, rolling conditions are set so that when mid-thickness temperature is T₁ °C or more, which is a recrystallization temperature range, average rolling reduction per pass is 3 % or more and cumulative rolling reduction ratio is 25 % or more, rolling is avoided at the partial recrystallization range temperature (T₁ °C to T₂ °C) at which recrystallization grains and coarse recovery grains would be generated, and further, at T₂ °C or less, which is a non-recrystallization temperature range, cumulative rolling reduction ratio is 30 % or more. The inventors discovered that these rolling conditions can sufficiently refine and homogenize the microstructure in the mid-thickness part, and crystal grain refinement and homogenization can occur to achieve the desired crystal grain size.

The present disclosure is based on these discoveries and further studies. Specifically, primary features of the present disclosure are described below.
[1] A steel plate having a thickness exceeding 100 mm and comprising a chemical composition containing (consisting of), in mass%, C: 0.03 % to 0.13 %, Si: 0.60 % or less, Mn: 0.9 % to 2.7 %, P: 0.050 % or less, S: 0.0050 % or less, Al: 0.002 % to 0.100 %, Ti: 0.002 % to 0.055 %, Nb: 0.005 % to 0.070 %, Ca: 0.0005 % to 0.0200 %, N: 0.0120 % or less, and O: 0.0070 % or less, with the balance being Fe and inevitable impurity, wherein the chemical composition satisfies Expressions (1) to (4) below, $1.50 \leq \left[Ti\right] / \left[N\right] \leq 5.00$ $0 \leq \left\{\left[Ca\right]-\left(0.18+130\left[Ca\right]\right)\times \left[O\right]\right\} / 1.25 / \left[S\right] \leq 1.50$ 0.280 % ≤ Ceq (= [C] + [Mn]/6 + ([Cu] + [Ni])/15 + ([Cr] + [Mo] + [V])/5) ≤ 0.500 % Pcm (= [C] + [Si]/30 + ([Mn] + [Cu] + [Cr])/20 + [Ni]/60 + [Mo]/ 15 + [V]/10 + 5[B]) ≤ 0.240 %
   where the square brackets in Expressions (1) to (4) indicate content in mass% of an element enclosed in the brackets and have a value of 0 when the element is not contained,
   in a mid-thickness part, average effective crystal grain size is 20 µm or less and maximum effective crystal grain size is 150 µm or less, and
   at a 1/2 thickness position, composite inclusions containing sulfides containing Ca and Mn and oxides containing Al and having a circle equivalent diameter of 0.1 µm or more are present at a number density of 25/mm² to 250/mm².
[2] The steel plate according to [1], wherein the chemical composition further contains, in mass%, at least one selected from the group consisting of Ni: 2.5 % or less, Cu: 2.0 % or less, Cr: 1.5 % or less, Mo: 1.5 % or less, V: 0.25 % or less, W: 0.45 % or less, B: 0.0045 % or less, REM: 0.025 % or less, and Mg: 0.005 % or less.
[3] A method of producing a steel plate, the method comprising:
   heating a material having the chemical composition defined in [1] or [2] to a temperature of 990 °C or more and 1210 °C or less; then rolling under rolling conditions including an average rolling reduction per pass of 3 % or more and a cumulative rolling reduction ratio of 25 % or more in a temperature range where mid-thickness temperature is T₁ °C or more as defined in Expression (5) below; rolling under rolling conditions including a cumulative rolling reduction ratio of 30 % or more in a temperature range where the mid-thickness temperature is T₂ °C or less as defined in Expression (6) below; and then cooling at an average cooling rate of 1.0 °C/s to 50.0 °C/s in the mid-thickness temperature to a cooling stop temperature of 600 °C or less,
      [Math. 1] ${T}_{1} = 174 log \left[sol.\left[Nb\right]\times \left(\left[C\right]+\frac{12}{14}\left[N\right]\right)\right] + 1444$ (Here, sol.[Nb] is derived from Expression (7))
      [Math. 2] ${T}_{2} = {T}_{1} - 75$
      [Math. 3] $sol . \left[Nb\right] = exp \left[2.3\left\{2.26-\frac{6770}{{T}_{0} + 273}-log\left(\left[C\right]+\frac{12}{14}\left[N\right]\right)\right\}\right]$
   and in Expressions (5) and (7), [C] and [N] represent mass% of C and N, respectively, T₀ represents heating temperature of the material in °C, and sol.[Nb] represents Nb solute in mass%, and sol.[Nb] ≤ [Nb] where [Nb] is the total Nb content in mass% in the steel plate.
[4] The method of producing a steel plate according to [3], wherein, after the cooling to the cooling stop temperature, a tempering treatment is performed at a temperature of 700 °C or less.

### (Advantageous Effect)

According to the present disclosure, a steel plate having high strength and excellent toughness of base metal and multilayer-fill-welded joint CTOD properties at low temperatures is provided, as well as a method of producing same.

### DETAILED DESCRIPTION

The reasons for limitations placed on the features of the present disclosure are explained below.

### [Chemical composition]

First, the reasons for limiting the chemical composition of the steel plate and the material to the ranges of the present disclosure are described. Hereinafter, "%" of each component means "mass%" unless otherwise specified.

### C: 0.03 % to 0.13 %

C is an element that increases hardenability and improves strength of steel. C content needs to be 0.03 % or more. However, the C content exceeding 0.13 % increases the hardness of C-enriched portions and degrades joint CTOD properties. The C content is therefore in the range from 0.03 % to 0.13 %. The C content is preferably 0.04 % or more. The C content is preferably 0.12 % or less. The C content is more preferably 0.06 % or more. The C content is more preferably 0.10 % or less.

### Si: 0.60 % or less

Si is also used as a deoxidizer, but is an element inevitably included as an impurity, and excessive Si content exceeding 0.60 % decreases joint CTOD properties. The Si content is therefore limited to an upper limit of 0.60 %. The upper limit is preferably 0.50 % or less. A lower limit is not particularly limited, but lowering Si excessively leads to increased refining time and higher costs, and therefore the lower limit of the Si content is preferably around 0.02 %. The Si content is more preferably 0.04 % or more.

### Mn: 0.9 % to 2.7 %

Mn is an element that has the effect of improving strength of the base metal and welded portion through improvement of hardenability of steel. To obtain these effects, addition of 0.9 % or more is required. However, addition exceeding 2.7 % not only decreases weldability, but also causes excessive hardenability, which reduces toughness of the base metal and welded portion, resulting in degradation of joint CTOD properties. The Mn content is therefore in the range from 0.9 % to 2.7 %. The Mn content is preferably 1.1 % or more. The Mn content is preferably 2.5 % or less. The Mn content is more preferably 1.2 % or more. The Mn content is more preferably 2.3 % or less.

### P: 0.050 % or less

P is an element that has a large effect of embrittling grain boundaries, and when added in large amounts decreases HAZ toughness and degrades joint CTOD properties. P content is therefore limited to 0.050 % or less. The P content is preferably 0.030 % or less. Decreasing P content as much as possible is desirable, and therefore a lower limit of the P content is not particularly limited. However, excessively low P content leads to increased refining time and higher costs. The P content is therefore preferably 0.001 % or more. The P content is more preferably 0.005 % or more.

### S: 0.0050 % or less

S is an element that degrades joint CTOD properties, and therefore an upper limit of S content is limited to 0.0050 %. The upper limit is preferably 0.0030 % or less. Decreasing S content as much as possible is desirable, and therefore a lower limit of the S content is not limited. However, excessively low S content leads to increased refining time and higher costs. The S content is therefore preferably 0.0001 % or more. The S content is more preferably 0.0005 % or more.

### Al: 0.002 % to 0.100 %

Al is an element required for formation of composite inclusions to improve toughness of multilayer-fill-welded HAZ and to improve joint CTOD properties, and needs to be added at 0.002 % or more. However excessive addition of more than 0.100 % causes the amount of composite inclusions to become excessive and joint CTOD properties in a low temperature range to degrade. The Al content is therefore in the range from 0.002 % to 0.100 %. The Al content is preferably 0.005 % or more. The Al content is preferably 0.090 % or less. The Al content is more preferably 0.020 % or more. The Al content is more preferably 0.075 % or less.

### Ti: 0.002 % to 0.055 %

Ti precipitates in steel as TiN. Precipitated TiN has an effect of inhibiting coarsening of austenite grains in the base metal and HAZ, refining HAZ microstructure and improving joint CTOD properties. To obtain these effects, addition of 0.002 % or more is required. However, when the Ti content exceeds 0.055 %, Ti nitrides coarsen and toughness of the heat-affected zone instead degrades, resulting in degradation of joint CTOD properties. The Ti content is therefore in the range from 0.002 % to 0.055 %. The Ti content is preferably 0.005 % or more. The Ti content is preferably 0.050 % or less. The Ti content is more preferably 0.010 % or more. The Ti content is more preferably 0.045 % or less.

### Nb: 0.005 % to 0.070 %

Nb is an element that broadens the non-recrystallization temperature range of austenite phase and has an effect of improving strength and toughness of base metal via efficient non-recrystallization range rolling to obtain a fine grain microstructure. When Nb is not added, the non-recrystallization temperature T₂ becomes too low, and the rolling temperature for non-recrystallization range rolling for fine grain formation becomes too low. Rolling at low temperatures increases the deformation resistance of the rolled material and increases load on the rolling mill, resulting in an increase in the number of rolling passes, which reduces production efficiency and makes it difficult to increase pass rolling reduction. As a result, appropriate introduction of strain to 1/2 t in steel plates having a thickness exceeding 100 mm becomes impossible, making obtaining desired properties difficult. To achieve such effects, the Nb content needs to be 0.005 % or more. However, when the Nb content exceeds 0.070 %, joint CTOD properties degrade. The Nb content is therefore in the range from 0.005 % to 0.070 %. The Nb content is preferably 0.010 % or more. The Nb content is preferably 0.060 % or less. The Nb content is more preferably 0.015 % or more. The Nb content is more preferably 0.050 % or less.

### Ca: 0.0005 % to 0.0200 %

Ca is an element that improves toughness of multilayer-fill-welded HAZ and improves joint CTOD properties by forming acid sulfides that are highly stable at high temperatures. To achieve such effects, the Ca content needs to be 0.0005 % or more. However, the content exceeding 0.0200 % causes excessive precipitation of acid sulfides, which instead degrades joint CTOD properties. The Ca content is therefore in the range from 0.0005 % to 0.0200 %. The Ca content is preferably 0.0010 % or more. The Ca content is preferably 0.0170 % or less. The Ca content is more preferably 0.0015 % or more. The Ca content is more preferably 0.0150 % or less.

### N: 0.0120 % or less

N is an element that reduces HAZ toughness and degrades joint CTOD properties, and therefore an upper limit of N content is limited to 0.0120 %. Decreasing N content as much as possible is desirable, and therefore a lower limit of the N content is not limited. However, excessively low N content leads to increased refining time and higher costs. The N content is therefore preferably 0.0005 % or more. The N content is more preferably 0.0020 % or more. The N content is more preferably 0.0110 % or less. The N content is more preferably 0.0030 % or more. The N content is more preferably 0.0090 % or less.

### O: 0.0070 % or less

O is an element that decreases HAZ toughness and degrades joint CTOD properties, and therefore an upper limit of O content is limited to 0.0070 %. Decreasing O content as much as possible is desirable, and therefore a lower limit of the O content is not limited. However, excessively low O content leads to increased refining time and higher costs. The O content is therefore preferably 0.0005 % or more. The O content is more preferably 0.0010 % or more. The O content is more preferably 0.0060 % or less. The O content is even more preferably 0.0015 % or more. The O content is even more preferably 0.0055 % or less.

The chemical composition of the steel plate according to an embodiment consists of the required elements described above, with the balance being Fe and inevitable impurity.

Further, according to another embodiment, for the purpose of further improving strength, toughness of base metal, joint toughness, and the like, the chemical composition may further contain at least one optional element selected from the group consisting of Ni, Cu, Cr, Mo, V, W, B, REM, and Mg, in a quantity indicated below.

### Ni: 2.5 % or less

Ni is an element which can increase strength of a steel plate without greatly degrading toughness of both base metal and joints. However, when Ni content exceeds 2.5 %, production costs and environmental impact increase. The Ni content is therefore limited to 2.5 % or less. The Ni content is more preferably 2.0 % or less. However, when added, the Ni content is preferably 0.1 % or more.

### Cu: 2.0 % or less

Cu is an element that can increase strength of steel plates without significantly degrading toughness of the base metal and joints. However, when Cu content exceeds 2.0 %, surface cracks caused by a Cu-enriched layer that forms just below scale become a problem. The Cu content is therefore limited to 2.0 % or less. The Cu content is more preferably 1.8 % or less. However, when added, the Cu content is preferably 0.05 % or more. The Cu content is more preferably 0.1 % or more.

### Cr: 1.5 % or less

Cr is an element that has an effect of increasing strength of steel through improving hardenability. However, Cr content exceeding 1.5 % degrades joint CTOD properties, and therefore the Cr content is limited to 1.5 % or less. The Cr content is more preferably 1.3 % or less. However, when added, the Cr content is preferably 0.05 % or more. The Cr content is more preferably 0.1 % or more.

### Mo: 1.5 % or less

Mo is an element that has an effect of increasing strength of steel through improving hardenability. However, Mo content exceeding 1.5 % degrades joint CTOD properties, and therefore the Mo content is limited to 1.5 % or less. The Mo content is more preferably 1.3 % or less. However, when added, the Mo content is preferably 0.05 % or more. The Mo content is more preferably 0.1 % or more.

### V: 0.25 % or less

V is an element that improves strength of the base metal, but when V content exceeds 0.25 %, HAZ toughness decreases and joint CTOD properties degrade, and therefore the V content is limited to 0.25 % or less. The V content is more preferably 0.20 % or less. However, when added, the V content is preferably 0.01 % or more. The V content is more preferably 0.03 % or more.

### W: 0.45 % or less

W is an element that improves strength of the base metal, but when W content exceeds 0.45 %, HAZ toughness decreases and joint CTOD properties degrade, and therefore the W content is limited to 0.45 % or less. The W content is more preferably 0.40 % or less. However, when added, the W content is preferably 0.05 % or more. The W content is more preferably 0.15 % or more.

### B: 0.0045 % or less

B is an element that can improve hardenability and thereby strength of a steel plate when contained in trace amounts. However, when B content exceeds 0.0045 %, HAZ toughness decreases and joint CTOD properties degrade, and therefore the B content is limited to 0.0045 % or less. The B content is more preferably 0.0040 % or less. However, when added, the B content is preferably 0.0005 % or more. The B content is more preferably 0.0010 % or more.

### REM: 0.025 % or less

Rare earth metals (REM) suppress austenite grain growth in the HAZ and improve HAZ toughness by forming acid sulfide inclusions, but when REM content exceeds 0.025 %, toughness of base metal and HAZ toughness are instead decreased and joint CTOD properties degrade. The REM content is therefore limited to 0.025 % or less. The REM content is more preferably 0.020 % or less. However, when added, the REM content is preferably 0.001 % or more. The REM content is more preferably 0.010 % or more.

### Mg: 0.005 % or less

Mg is an element that suppresses growth of austenite grains in the heat-affected zone by forming oxide inclusions and improves toughness of the heat-affected zone. However, when Mg content exceeds 0.005 %, the effect of addition saturates, and an effect commensurate with content cannot be expected, which is economically disadvantageous. The Mg content is therefore limited to 0.005 % or less. The Mg content is more preferably 0.004 % or less. However, when added, the Mg content is preferably 0.0005 % or more. The Mg content is more preferably 0.001 % or more.

According to the present disclosure, chemical composition of the steel plate and the material is required to further satisfy each of the four conditions described below. $1.50 \leq \left[Ti\right] / \left[N\right] \leq 5.00$ [Ti] / [N] controls the amount of solute N and the precipitation state of TiN in the HAZ. When [Ti] / [N] is less than 1.50, HAZ toughness degrades due to the presence of solute N that is not fixed as TiN, and joint CTOD properties degrade. On the other hand, when [Ti] / [N] is more than 5.00, HAZ toughness degrades due to precipitation of coarse TiN, and joint CTOD properties degrade. The [Ti] / [N] range is therefore 1.50 to 5.00. The [Ti] / [N] range is preferably 1.80 or more. The [Ti] / [N] range is preferably 4.50 or less. The [Ti] / [N] range is more preferably 2.00 or more. The [Ti] / [N] range is more preferably 4.00 or less.$0 \leq \left\{\left[Ca\right]-\left(0.18+130\left[Ca\right]\right)\times \left[O\right]\right\} / 1.25 / \left[S\right] \leq 1.50$

{[Ca] - (0.18 + 130 [Ca]) x [O]} / 1.25 / [S] is the atomic concentration ratio (ACR) of Ca, O, and S in steel. When the ACR is less than 0, the main form of sulfide inclusions is MnS. MnS has a low melting point and melts in the vicinity of the weld line during welding, and therefore the effect of suppressing austenite grain coarsening in the vicinity of the weld line and the effect of transformation during cooling after welding cannot be obtained, resulting in joint CTOD properties degrading. On the other hand, when the ACR exceeds 1.50, the main form of sulfide inclusions is CaS. CaS does not form a Mn-poor layer around CaS, which is necessary to form nucleation sites, and therefore the nucleation site effect is not obtained and joint CTOD properties are degraded. Accordingly, the ACR range is 0 or more and 1.50 or less. The ACR range is preferably 0.20 or more. The ACR range is preferably 1.40 or less. The ACR range is more preferably 0.40 or more. The ACR range is more preferably 1.20 or less.

### Ceq: 0.280 % or more and 0.500 % or less

When the equivalent carbon content Ceq, defined by the following Expression (3), is increased, microstructure having poor toughness such as martensite austenite constituent and bainite increases in HAZ microstructure, and therefore HAZ toughness degrades. That is, when Ceq is more than 0.500 %, the HAZ matrix itself suffers toughness degradation, and therefore even with HAZ toughness improvement techniques through composite inclusions, the required joint CTOD properties cannot be satisfied. On the other hand, when Ceq is less than 0.280 %, the target strength cannot be secured. The Ceq range is therefore 0.280 % to 0.500 %. The Ceq range is preferably 0.300 % or more. The Ceq range is preferably 0.490 % or less. The Ceq range is more preferably 0.320 % or more. The Ceq range is more preferably 0.480 % or less. Ceq (%) = [C] + [Mn]/6 + ([Cu] + [Ni])/15 + ([Cr] + [Mo] + [V])/ 5

### Pcm: 0.240 % or less

When the weld cracking parameter Pcm defined by the following Expression (4) is increased, microstructure having poor toughness such as martensite austenite constituent and bainite increases in HAZ microstructure, and therefore HAZ toughness degrades. That is, when Pcm exceeds 0.240 %, the HAZ matrix itself suffers toughness degradation, and therefore the required joint CTOD properties cannot be obtained. Pcm is therefore 0.240 % or less. Pcm is preferably 0.230 % or less. Pcm is more preferably 0.210 % or less. A lower limit is not particularly limited. Excessive attempts to decrease Pcm result in too low a Ceq value, and therefore the lower limit is preferably about 0.140 %. Pcm is more preferably 0.155 % or more. Pcm (%) = [C] + [Si]/30 + ([Mn] + [Cu] + [Cr])/20 + [Ni]/60 + [Mo]/15 + [V]/10 + 5[B]

The square brackets [] in Expressions (1) to (4) indicate content in mass% of an element enclosed in the brackets and have a value of 0 when the element is not contained.

### [Average effective crystal grain size]

Average effective crystal grain size at mid-thickness part (meaning a range of 10 % of the thickness of the steel plate towards each surface, centered at the 1/2 thickness position of the steel plate): 20 µm or less

According to the present disclosure, average effective crystal grain size of microstructure in the mid-thickness part of the steel plate having a thickness exceeding 100 mm is 20 µm or less. Crystal grains in the mid-thickness part in which segregation is easily caused are refined as described above to improve base metal toughness, thereby increasing joint CTOD properties at SC/ICHAZ boundaries. The smaller the average effective crystal grain size, the more advantageous, and therefore a lower limit of the average effective crystal grain size is not particularly limited. Typically, the lower limit is about 1 µm.

Here, "effective crystal grain size" is defined as the circle equivalent diameter of a crystal grain surrounded by grain boundaries of crystal grains having an orientation difference of 15° or more, that is, large-angle grain boundaries. Further, the average effective crystal grain size in the mid-thickness part can be measured by a method described in the following EXAMPLES section.

### [Maximum effective crystal grain size]

According to the present disclosure, the maximum effective crystal grain size of the microstructure in the mid-thickness part is 150 µm or less. For example, even when the average effective crystal grain size is 20 µm or less, when coarse crystal grains having an effective crystal grain size exceeding 150 µm are mixed into the mid-thickness part, the coarse crystal grains become fracture origins and lead to a decrease in base metal strength, base metal toughness, and SCHAZ toughness in the mid-thickness part. The maximum effective crystal grain size is therefore 150 µm or less. The maximum effective crystal grain size can be measured by the method described in the EXAMPLES section below.

### [Composite inclusions]

The present disclosure limits the number density at the 1/2 thickness position of composite inclusions containing sulfides containing Ca and Mn and oxides containing Al and having a circle equivalent diameter of 0.1 µm or more to a range from 25/mm² to 250/mm².

When Mn-containing sulfides are formed, Mn-poor regions forming around the composite inclusions are effective as nucleation sites. Further, the inclusion of Ca in such sulfides results in a high melting point and allows the inclusions to remain at the temperatures reached by the HAZ in the vicinity of the weld line. As a result, the austenite grain growth suppression and nucleation site effects are exhibited, and joint CTOD properties are improved. In order to fully exhibit the above effect, the number density of composite inclusions at the 1/2 thickness position needs to be 25/mm² or more. On the other hand, the presence of excessive amounts of composite inclusions can degrade joint CTOD properties. Therefore, the number density of composite inclusions having a circle equivalent diameter of 0.1 µm or more at the 1/2 thickness position is 250/mm² or less. The number density is preferably 30/mm² or more. The number density is preferably 215/mm² or less. The number density is more preferably 50/mm² or more. The number density is more preferably 200/mm² or less. The number density can be measured by the method described in the EXAMPLES section below.

Here, the frequency of measurement of average effective crystal grain size, maximum effective crystal grain size, and composite inclusions may be such that one or two cross-sections at the mid-thickness part of any one steel plate are measured among steel plates produced under the same material smelting conditions and rolling conditions. As long as the material steelmaking method and rolling conditions are not changed, the crystal grain size and inclusion number density are highly reproducible, and therefore measurement results at the above measurement frequency are representative of the whole.

### [Production method]

Next, the reasons for limiting each condition in the method of producing the steel plate according to the present disclosure are explained below. In the following description, "temperature" means temperature at the mid-thickness part, unless otherwise noted. Further, temperature at the mid-thickness part may be measured as described in the following EXAMPLES section. However, for example, on an actual production line, temperature at a surface of a steel plate may be measured using a radiation thermometer and temperature at the mid-thickness part may be determined by heat transfer calculation.

### • Material heating conditions

According to the present disclosure, a method of preparing the material is not particularly limited, and any known steelmaking method may be applied, such as a converter, an electric furnace, a vacuum melting furnace, and the like. The material may be produced, for example, by a continuous casting method. Further, molten steel from which the material is produced may be further subjected to secondary refining such as ladle refining.

The material having the chemical composition and produced as described above is heated to a temperature of 990 °C or more and 1210 °C or less. When the heating temperature is lower than 990 °C, the following conditions of hot rolling cannot be met, and a sufficient effect cannot be obtained. On the other hand, when the heating temperature is higher than 1210 °C, austenite grains become coarse and the desired fine grain microstructure cannot be obtained after controlled rolling. For these reasons, the range of the heating temperature is 990 °C or more to 1210 °C or less. The temperature is preferably 1010 °C or more. The temperature is preferably 1190 °C or less. The temperature is more preferably 1030 °C or more. The temperature is more preferably 1170 °C or less.

### • Hot rolling conditions

According to the present disclosure, in hot rolling, it is important to control the rolling conditions for both the recrystallization temperature range defined as the T₁ temperature or more, according to Expression (5) below, and the non-recrystallization temperature range defined as the T₂ temperature or less, according to Expression (6) below. It is also important to avoid rolling at the partial recrystallization temperature range (T₁ °C to T₂ °C) where recrystallization grains and coarse recovered grains are generated. The recrystallization temperature range and the non-recrystallization temperature range vary depending on the composition, and therefore clarifying the recrystallization temperature range and the non-recrystallization temperature range for each chemical composition of steel by Expressions (5) and (6) is important.
[Math. 4] ${T}_{1} = 174 log \left[sol.\left[Nb\right]\times \left(\left[C\right]+\frac{12}{14}\left[N\right]\right)\right] + 1444$ (Here, sol.[Nb] is derived from Expression (7))
[Math. 5] ${T}_{2} = {T}_{1} - 75$
[Math. 6] $sol . \left[Nb\right] = exp \left[2.3\left\{2.26-\frac{6770}{{T}_{0} + 273}-log\left(\left[C\right]+\frac{12}{14}\left[N\right]\right)\right\}\right]$ (In Expressions (5) and (7), [C] and [N] represent mass% of C and N, respectively, T₀ represents heating temperature of the material in °C, and sol.[Nb] represents Nb solute in mass%. However, when [Nb] is the total Nb content in mass% in the steel plate, sol.[Nb] is always sol.[Nb] ≤ [Nb]. Accordingly, when the result of the calculation in Expression (7) is that sol.[Nb] > [Nb], then sol.[Nb] in Expression (7) is the value of [Nb].)

Rolling in the recrystallization temperature range defined as the mid-thickness temperature being the T₁ temperature or more is carried out with an average rolling reduction per pass of 3 % or more and cumulative rolling reduction ratio of 25 % or more.

The purpose of rolling in the recrystallization temperature range is to refine the microstructure by recrystallization, homogenize microstructure, and to refine and disperse coarse inclusions, even in steel plates having a thickness exceeding 100 mm. When hot rolling is performed in the partial recrystallization temperature range where the mid-thickness temperature is T₁ °C to T₂ °C, a mixed-grain-size microstructure of recrystallized grains and coarse recovered grains is formed and the desired uniformly-sized grain microstructure cannot be obtained. Therefore, it is necessary to roll at the mid-thickness temperature of T₁ °C or more while avoiding rolling at the mid-thickness temperature of T₁ °C to T₂ °C. When the average rolling reduction per pass is less than 3 %, it is not possible to introduce sufficient strain into the mid-thickness part in a steel plate having a thickness exceeding 100 mm thick, and the mid-thickness part microstructure cannot be sufficiently refined. Further, even when the average rolling reduction per pass is 3 % or more, when cumulative rolling reduction ratio is less than 25 %, recrystallization does not progress sufficiently and uniform microstructure cannot be obtained. For this reason, rolling in the recrystallization temperature range is performed with an average rolling reduction per pass of 3 % or more and a cumulative rolling reduction ratio of 25 % or more. The cumulative rolling reduction ratio is preferably 30 % or more. The cumulative rolling reduction ratio is more preferably 35 % or more.

Subsequent rolling in the non-recrystallization temperature range, where the mid-thickness temperature is defined as the T₂ temperature or less, is performed so that the cumulative rolling reduction ratio is 30 % or more.

Rolling when the mid-thickness temperature is in the non-recrystallization temperature range prevents recrystallization in the steel microstructure, and therefore the strain introduced by rolling is not consumed by recrystallization but accumulates and becomes the driving force for nucleation in the subsequent cooling process. As a result, the finally obtained steel plate can have a refined microstructure. On the other hand, when the cumulative rolling reduction ratio in the non-recrystallization temperature range of the mid-thickness part is less than 30 %, the crystal grain refinement effect is insufficient and the average effective crystal grain size in the mid-thickness part cannot be made to be 20 µm or less. For this reason, rolling in the non-recrystallization temperature range is performed with a cumulative rolling reduction ratio of 30 % or more. The cumulative rolling reduction ratio is preferably 35 % or more. The cumulative rolling reduction ratio is more preferably 40 % or more.

The conditions for rolling in the non-recrystallization temperature range are not particularly limited. A larger average rolling reduction per pass (average of rolling reduction in each pass) is preferable, and specifically, the average rolling reduction per pass is preferably 3 % or more.

### [Cooling]

After completion of the hot rolling, the obtained hot-rolled steel plate is cooled. The cooling can be done by any method as long as the conditions described below are met. For example, the cooling can be done by water cooling.

### Average cooling rate: 1.0 °C/s to 50.0 °C/s

When the average cooling rate at mid-thickness is less than 1.0 °C/s, a coarse ferrite phase is generated in the matrix microstructure, resulting in a decrease in matrix strength and toughness of base metal and degradation of SC/ICHAZ CTOD properties. On the other hand, when the average cooling rate is greater than 50.0 °C/s, an increase in hard bainite phase increases base metal strength and degrades SC/ICHAZ CTOD properties. The average cooling rate at the mid-thickness position is therefore 1.0 °C/s to 50.0 °C/s. The average cooling rate at the mid-thickness position is preferably 1.2 °C/s or more. The average cooling rate is preferably 45 °C/s or less. The average cooling rate is more preferably 1.5°C/s or more. The average cooling rate is more preferably 40°C/s or less.

Regarding the temperature measurement range of the cooling rate, when the cooling stop temperature is 500 °C or less, the range is 700 °C to 500 °C. When the cooling stop temperature is greater than 500 °C, the range is 700 °C to the cooling stop temperature.

### Cooling stop temperature: 600 °C or less

In the cooling, the hot-rolled steel plate is cooled to a cooling stop temperature where the mid-thickness temperature is 600 °C or less. When the cooling stop temperature is greater than 600 °C, microstructure after transformation becomes coarse, resulting in insufficient base metal strength, a decrease in base metal toughness, and degradation of SC/ICHAZ CTOD properties. The cooling stop temperature at the mid-thickness temperature is therefore 600 °C or less. The cooling stop temperature is preferably 580 °C or less. The cooling stop temperature is more preferably 560 °C or less. A lower limit of the cooling stop temperature is not particularly limited. The lower limit is preferably about 200 °C.

### [Tempering treatment]

### Tempering Temperature: 700 °C or less

After the cooling stop, the steel plate may be subjected to tempering treatment. Tempering treatment can further improve base metal toughness. At this time, a tempering temperature higher than 700 °C generates a coarse ferrite phase, thus degrading base metal toughness and SCHAZ toughness. Accordingly, the tempering temperature at the mid-thickness temperature is 700 °C or less. The tempering temperature is more preferably 650 °C or less. A lower limit of the tempering temperature is not particularly limited as long as the effect of improving base metal toughness can be obtained. The lower limit may be around 300 °C.

In the production method according to the present disclosure, anything not described herein may follow a conventional method.

### EXAMPLES

More detailed description is given below based on examples. The following examples merely represent preferred examples, and the present disclosure is not limited to these examples.

Material having a chemical composition listed in Table 1 was used to produce steel plates under the production conditions listed in Table 2. Rolling at T₁ °C or more was performed with an average rolling reduction per pass ≥ 3 %. During hot rolling, a thermocouple was attached in a central position in the longitudinal direction, width direction, and thickness direction of each steel material to be hot rolled to measure the temperature of the mid-thickness part. At the same time, surface temperature of the steel material was measured with a radiation thermometer.

Average effective crystal grain size, maximum effective crystal grain size, number density of composite inclusions containing sulfides containing Ca and Mn and oxides containing Al, yield stress, toughness, and CTOD properties were measured for each of the steel plates obtained by the following methods.

### [Average effective crystal grain size and maximum effective crystal grain size]

A sample was collected from each obtained steel plate so that a measurement position was located at a central position in the longitudinal direction, width direction, and thickness direction of the steel plate, so as to include the mid-thickness part. Then, after mirror polishing a surface of the sample, electron backscatter pattern (EBSP) analysis was performed under the following conditions. From an obtained crystal orientation map, a circle equivalent diameter of a microstructure surrounded by a large-angle grain boundary having an orientation difference of 15° or more from adjacent crystal grains was determined, and an average of the circle equivalent diameters in the following analysis region was defined as an average effective crystal grain size. The maximum value of circle equivalent diameter obtained was defined as the maximum effective grain size.

EBSP analysis conditions
- Analysis region: 1 mm x 1 mm area at mid-thickness
- Step size: 0.4 µm

### [Number density of composite inclusions containing sulfides containing Ca and Mn and oxides containing Al]

Samples were taken from the center of the steel plate in the longitudinal, width, and thickness directions, and mirror polished, finishing with diamond buffing + alcohol. Then, using a field emission scanning electron microscope (FE-SEM), composite inclusions having a circle equivalent diameter of 0.1 µm or more in the 1 mm × 1 mm evaluation area, the center of which is the center of the area, were identified by EDX (energy dispersive X-ray spectroscopy) analysis, and the number density of the composite inclusions was also evaluated. Evaluation of inclusion type was performed such that an inclusion was judged to contain an element when the chemical composition of the inclusion, quantified by the ZAF method, contained 3 % or more of the element in terms of atomic fraction.

### [Yield stress]

Tensile tests were conducted according to EN 10002-1 to determine yield stress (YS) at 1/2 positions of thickness (t) of each steel plate. For each tensile test, a round bar tensile test piece having a parallel portion diameter of 14 mm and a parallel portion length of 70 mm was used, the test pieces being taken parallel to the plate transverse direction from 1/2 positions of plate thickness. When the upper yield point appeared in the tensile test, the upper yield point was used as the yield stress, and when the upper yield point did not appear, the 0.2 % proof stress was used as the yield stress.

### [Base metal toughness]

Three V-notch test pieces as specified in Japanese Industrial Standard JIS Z2242 were taken from the 1/2 thickness position of the steel plate so that the longitudinal direction of each test piece was perpendicular to the rolling direction of the plate. The absorbed energy vE-_{40 °C} at -40 °C was measured by the Charpy impact test. The base metal toughness was considered to be good when the average vE-_{40 °C} of three such test pieces was 100 J or more.

Next, each steel plate was used to produce a multilayer-fill-welded joint. Each obtained multilayer-fill-welded joint was subjected to a joint CTOD test to measure the amount of crack opening displacement in the CGHAZ and the amount of crack opening displacement in the SC/ICHAZ. The conditions for production of the multilayer-fill-welded joints and the conditions of the joint CTOD tests are described below.

### [Joint CTOD test]

Welded joints used for the joint CTOD tests were produced by submerged arc welding (multilayer fill welding) with K groove geometry and heat input of 5.0 kJ/mm. The test method was based on BS EN10225-4 (2019), and the crack opening displacement (CTOD value (δ)) was evaluated at the test temperature of -20 °C using test pieces each having a square cross-section of t x t (where t is plate thickness).

A test where the notch position was set as the CGHAZ on the linear side of the K groove and a test where the notch position was set at the SC/ICHAZ boundary were conducted, and the δ of the CGHAZ and the δ of the SC/ICHAZ boundary were measured, respectively. For each steel plate, the test was performed for three test pieces per notch position and the lowest value measured was taken as δ.

A higher CTOD value (δ) indicates that a brittle crack is less likely to occur.

After the tests, on a fracture surface of the test piece, the end of a fatigue precrack was confirmed to be located both in the CGHAZ and at the SC/ICHAZ boundary specified by EN10225-4 (2019). In the case of joint CTOD test of multilayer fill welding, even when a notch position is located in the CGHAZ, a certain amount of the ICCGHAZ is also included, and therefore the test result reflects toughness of both the CGHAZ and the ICCGHAZ.

The measurement results are listed in Table 2.

### [Table 1]

**Table 1**

| Ref. ID | Chemical composition (mass%) | | | | | | | | | | | | [Ti]/[N] | ACR (Expression (2)) | Ceq (%) | Pcm (%) | Classification |
|---|---|---|---|---|---|---|---|---|---|---|---|---|---|---|---|---|---|
| | C | Si | Mn | P | S | Al | Ti | Nb | Ca | N | O | Other | | | | | |
| A | 0.03 | 0.29 | 2.7 | 0.008 | 0.0005 | 0.055 | 0.021 | 0.025 | 0.0067 | 0.0048 | 0.0059 | - | 4.38 | 0.80 | 0.480 | 0.175 | Example |
| B | 0.06 | 0.07 | 1.6 | 0.011 | 0.0010 | 0.022 | 0.053 | 0.012 | 0.0080 | 0.0106 | 0.0054 | - | 5.00 | 1.13 | 0.327 | 0.142 | Example |
| C | 0.12 | 0.10 | 1.7 | 0.027 | 0.0019 | 0.062 | 0.012 | 0.015 | 0.0008 | 0.0042 | 0.0020 | - | 2.86 | 0.10 | 0.403 | 0.208 | Example |
| D | 0.04 | 0.32 | 1.8 | 0.009 | 0.0038 | 0.093 | 0.013 | 0.027 | 0.0025 | 0.0040 | 0.0045 | - | 3.25 | 0.05 | 0.340 | 0.141 | Example |
| E | 0.06 | 0.12 | 1.9 | 0.019 | 0.0049 | 0.047 | 0.004 | 0.066 | 0.0058 | 0.0025 | 0.0027 | - | 1.60 | 0.54 | 0.377 | 0.159 | Example |
| F | 0.13 | 0.58 | 0.9 | 0.047 | 0.0021 | 0.036 | 0.014 | 0.006 | 0.0190 | 0.0037 | 0.0070 | - | 3.78 | 0.17 | 0.280 | 0.194 | Example |
| G | 0.07 | 0.29 | 1.5 | 0.023 | 0.0022 | 0.040 | 0.018 | 0.040 | 0.0023 | 0.0113 | 0.0038 | - | 1.59 | 0.17 | 0.320 | 0.155 | Example |
| H | 0.09 | 0.05 | 1.6 | 0.024 | 0.0045 | 0.075 | 0.028 | 0.059 | 0.0135 | 0.0074 | 0.0052 | - | 3.78 | 0.61 | 0.357 | 0.172 | Example |
| I | 0.04 | 0.20 | 2.1 | 0.039 | 0.0029 | 0.035 | 0.019 | 0.031 | 0.0048 | 0.0084 | 0.0029 | Ni:1.0, Cu:0.3, V:0.10, Mg:0.004 | 2.26 | 0.68 | 0.497 | 0.193 | Example |
| J | 0.08 | 0.42 | 1.4 | 0.038 | 0.0008 | 0.031 | 0.008 | 0.018 | 0.0025 | 0.0027 | 0.0044 | Ni:0.4, Cr:0.3, Mo:0.3, B:0.0040 | 2.96 | 0.28 | 0.460 | 0.226 | Example |
| K | 0.06 | 0.03 | 1.9 | 0.016 | 0.0011 | 0.034 | 0.025 | 0.024 | 0.0058 | 0.0054 | 0.0055 | Cu:1.5, W:0.15, REM:0.022 | 4.63 | 0.48 | 0.477 | 0.231 | Example |
| L | 0.04 | 0.10 | 1.1 | 0.010 | 0.0042 | 0.031 | 0.026 | 0.016 | 0.0092 | 0.0072 | 0.0013 | Cr:1.3, Mg:0.001 | 3.61 | 1.41 | 0.483 | 0.163 | Example |
| M | 0.06 | 0.08 | 1.5 | 0.012 | 0.0040 | 0.089 | 0.012 | 0.027 | 0.0146 | 0.0049 | 0.0036 | Ni:2.2, V:0.20, W:0.40, B:0.0020 | 2.45 | 1.42 | 0.497 | 0.204 | Example |
| N | 0.05 | 0.09 | 1.0 | 0.007 | 0.0010 | 0.003 | 0.014 | 0.025 | 0.0025 | 0.0076 | 0.0020 | Cu:0.2, Mo:1.3, REM:0.010 | 1.84 | 1.19 | 0.490 | 0.200 | Example |
| O | 0.08 | 0.12 | 2.0 | 0.041 | 0.0026 | 0.037 | 0.018 | 0.010 | 0.0004 | 0.0072 | 0.0011 | - | 2.50 | 0.04 | 0.413 | 0.184 | Comparative Example |
| P | 0.04 | 0.16 | 1.9 | 0.044 | 0.0046 | 0.039 | 0.012 | 0.017 | 0.0210 | 0.0031 | 0.0049 | - | 3.87 | 1.17 | 0.357 | 0.140 | Comparative Example |
| Q | 0.03 | 0.42 | 0.9 | 0.046 | 0.0034 | 0.083 | 0.021 | 0.044 | 0.0081 | 0.0051 | 0.0063 | Cr:1.6, W:0.22, B:0.0020 | 4.12 | 0.08 | 0.500 | 0.179 | Comparative Example |
| R | 0.09 | 0.22 | 0.8 | 0.045 | 0.0014 | 0.065 | 0.009 | 0.054 | 0.0030 | 0.0058 | 0.0023 | Ni:1.5 | 1.55 | 0.97 | 0.323 | 0.162 | Comparative Example |
| S | 0.03 | 0.26 | 0.9 | 0.021 | 0.0044 | 0.048 | 0.033 | 0.067 | 0.0042 | 0.0070 | 0.0030 | Mo:1.6, REM:0.011, Mg:0.003 | 4.71 | 0.37 | 0.500 | 0.190 | Comparative Example |
| T | 0.05 | 0.57 | 2.5 | 0.031 | 0.0027 | 0.034 | 0.048 | 0.027 | 0.0124 | 0.0101 | 0.0050 | Cr:0.1, V:0.05, W:0.48, B:0.0040 | 4.75 | 1.02 | 0.497 | 0.224 | Comparative Example |
| U | 0.11 | 0.24 | 1.7 | 0.020 | 0.0030 | 0.010 | 0.015 | 0.004 | 0.0069 | 0.0079 | 0.0057 | - | 1.90 | 0.20 | 0.393 | 0.203 | Comparative Example |
| V | 0.14 | 0.26 | 1.2 | 0.023 | 0.0047 | 0.062 | 0.013 | 0.045 | 0.0012 | 0.0061 | 0.0016 | - | 2.13 | 0.11 | 0.340 | 0.209 | Comparative Example |
| W | 0.08 | 0.49 | 1.5 | 0.020 | 0.0053 | 0.082 | 0.008 | 0.036 | 0.0018 | 0.0019 | 0.0031 | - | 4.21 | 0.08 | 0.330 | 0.171 | Comparative Example |
| X | 0.07 | 0.23 | 2.0 | 0.055 | 0.0017 | 0.019 | 0.041 | 0.043 | 0.0116 | 0.0092 | 0.0061 | - | 4.46 | 0.61 | 0.403 | 0.178 | Comparative Example |
| Y | 0.08 | 0.51 | 2.3 | 0.032 | 0.0032 | 0.047 | 0.057 | 0.023 | 0.0069 | 0.0120 | 0.0022 | - | 4.75 | 1.13 | 0.463 | 0.212 | Comparative Example |
| Z | 0.10 | 0.16 | 1.4 | 0.046 | 0.0018 | 0.046 | 0.010 | 0.080 | 0.0051 | 0.0025 | 0.0028 | - | 4.00 | 1.22 | 0.333 | 0.175 | Comparative Example |
| AA | 0.02 | 0.44 | 2.6 | 0.046 | 0.0012 | 0.043 | 0.016 | 0.042 | 0.0037 | 0.0049 | 0.0026 | - | 3.27 | 1.32 | 0.453 | 0.165 | Comparative Example |
| AB | 0.05 | 0.63 | 2.5 | 0.048 | 0.0010 | 0.096 | 0.007 | 0.059 | 0.0040 | 0.0035 | 0.0040 | - | 2.00 | 0.96 | 0.467 | 0.196 | Comparative Example |
| AC | 0.12 | 0.08 | 1.3 | 0.025 | 0.0010 | 0.085 | 0.037 | 0.047 | 0.0034 | 0.0083 | 0.0043 | Ni:0.9, Cr:0.2, Mo:0.2, W:0.15, REM:0.027, Mg:0.002 | 4.46 | 0.58 | 0.477 | 0.226 | Comparative Example |
| AD | 0.04 | 0.21 | 2.0 | 0.012 | 0.0028 | 0.019 | 0.046 | 0.030 | 0.0071 | 0.0098 | 0.0059 | Cu:0.1, Mo:0.2, V:0.26 | 4.69 | 0.17 | 0.472 | 0.191 | Comparative Example |
| AE | 0.10 | 0.09 | 1.5 | 0.035 | 0.0028 | 0.110 | 0.015 | 0.061 | 0.0033 | 0.0036 | 0.0018 | - | 4.17 | 0.63 | 0.350 | 0.178 | Comparative Example |
| AF | 0.13 | 0.58 | 1.5 | 0.018 | 0.0043 | 0.001 | 0.038 | 0.041 | 0.0022 | 0.0089 | 0.0031 | - | 4.27 | 0.14 | 0.380 | 0.224 | Comparative Example |
| AG | 0.05 | 0.08 | 1.8 | 0.044 | 0.0029 | 0.028 | 0.001 | 0.038 | 0.0140 | 0.0006 | 0.0055 | - | 1.67 | 0.83 | 0.350 | 0.143 | Comparative Example |
| AH | 0.03 | 0.34 | 2.8 | 0.037 | 0.0037 | 0.061 | 0.053 | 0.021 | 0.0064 | 0.0112 | 0.0062 | - | 4.73 | 0.03 | 0.497 | 0.181 | Comparative Example |
| AI | 0.05 | 0.11 | 1.0 | 0.024 | 0.0023 | 0.035 | 0.021 | 0.060 | 0.0073 | 0.0051 | 0.0064 | Ni:0.6, Cu:1.5, V:0.08, B:0.0061, REM:0.017, Mg:0.004 | 4.12 | 0.03 | 0.373 | 0.227 | Comparative Example |
| AJ | 0.07 | 0.53 | 1.9 | 0.014 | 0.0017 | 0.055 | 0.044 | 0.025 | 0.0081 | 0.0130 | 0.0065 | - | 3.38 | 0.04 | 0.387 | 0.183 | Comparative Example |
| AK | 0.12 | 0.30 | 1.6 | 0.023 | 0.0046 | 0.059 | 0.035 | 0.022 | 0.0190 | 0.0086 | 0.0071 | - | 4.07 | 0.03 | 0.387 | 0.210 | Comparative Example |
| AL | 0.10 | 0.43 | 2.0 | 0.049 | 0.0045 | 0.094 | 0.026 | 0.025 | 0.013 5 | 0.0104 | 0.0021 | - | 2.50 | 1.68 | 0.433 | 0.214 | Comparative Example |
| AM | 0.12 | 0.59 | 2.1 | 0.049 | 0.0011 | 0.022 | 0.020 | 0.060 | 0.0097 | 0.0056 | 0.0064 | - | 3.57 | 0.35 | 0.470 | 0.245 | Comparative Example |
| AN | 0.07 | 0.37 | 1.2 | 0.033 | 0.0028 | 0.097 | 0.011 | 0.033 | 0.0118 | 0.0030 | 0.0043 | - | 3.67 | 1.27 | 0.270 | 0.142 | Comparative Example |
| AO | 0.09 | 0.37 | 1.6 | 0.038 | 0.0031 | 0.035 | 0.009 | 0.059 | 0.0102 | 0.0077 | 0.0061 | - | 1.17 | 0.26 | 0.357 | 0.182 | Comparative Example |
| AP | 0.10 | 0.15 | 2.5 | 0.044 | 0.0025 | 0.032 | 0.013 | 0.015 | 0.0133 | 0.0029 | 0.0047 | - | 4.48 | 1.38 | 0.517 | 0.230 | Comparative Example |
| AQ | 0.07 | 0.55 | 1.9 | 0.045 | 0.0016 | 0.095 | 0.018 | 0.019 | 0.0025 | 0.0038 | 0.0065 | - | 4.74 | -0.39 | 0.387 | 0.183 | Comparative Example |
| AR | 0.07 | 0.13 | 2.3 | 0.019 | 0.0049 | 0.068 | 0.044 | 0.062 | 0.0045 | 0.0087 | 0.0037 | - | 5.06 | 0.27 | 0.453 | 0.189 | Comparative Example |

| | | | | | | | | | | | | | | | | | |
|---|---|---|---|---|---|---|---|---|---|---|---|---|---|---|---|---|---|
| Note 1: the balance is Fe and inevitable impurity Note 2: underlining indicates value outside scope of present disclosure Note 3: AcR = {[Ca] - (0.18 + 130 [Ca]) x [O]} / 1.25 / [S] Ceq = [C] + [Mn] / 6 + ([Cu] + [Ni]) / 15 + ([Cr] + [Mo] + [V]) / 5 Pcm = [C] + [Si] / 30 + ([Mn] + [Cu] + [Cr]) / 20 + [Ni] / 60 + [Mo] / 15 + [V] / 10 + 5[B] | | | | | | | | | | | | | | | | | |

### [Table 2]

**Table 2**

| No. | Steel sample ID | Thickness (mm) | Production conditions | | | | | | | Measurement results | | | | | | | Classification |
|---|---|---|---|---|---|---|---|---|---|---|---|---|---|---|---|---|---|
| | | | Heating | Hot rolling | | | Cooling | | Tempering | Base metal properties | | | | | Welded portion properties | | |
| | | | Heating temp. (°C) | Cumulative rolling reduction ratio at T₁°C or more (%) | T₁°C to T₂°C rolling | Cumulative rolling reduction ratio at T₂°C or less (%) | Average cooling rate (°C/s) | Cooling stop temp. (°C) | Tempering temp. (°C) | Mid-thickness part average effective crystal grain size (µm) | Mid-thickness part maximum effective crystal grain size (µm) | 1/2 position composite inclusions ²) (per mm²) | 1/2 position YS (MPa) | 1/2 position vE__{40°}C (J) | -20°C CGHAZ δ (mm) | -20°C SC/ICHAZ boundary δ (mm) | |
| 1 | A | 101 | 1077 | 27 | No | 56 | 4.8 | 218 | - | 14 | 91 | 179 | 510 | 200 | 0.94 | 1.08 | Example |
| 2 | A | 146 | 1093 | 42 | No | 43 | 10.4 | 512 | 750 | 19 | 145 | 205 | 337 | 103 | 0.85 | 0.41 | Example |
| 3 | B | 150 | 1158 | 41 | No | 44 | 77 | 379 | 500 | 10 | 102 | 154 | 373 | 121 | 0.68 | 0.76 | Example |
| 4 | B | 135 | 1107 | 48 | No | 47 | 10.6 | 625 | - | 41 | 85 | 122 | 298 | 64 | 0.51 | 0.31 | Comparative Example |
| 5 | C | 137 | 975 | 14 | No | 59 | 1.3 | 541 | - | 27 | 170 | 17 | 426 | 89 | 0.33 | 0.38 | Comparative Example |
| 6 | C | 113 | 1068 | 38 | No | 48 | 4.2 | 344 | - | 14 | 98 | 215 | 447 | 123 | 1.16 | 0.74 | Example |
| 7 | D | 129 | 1195 | 31 | No | 33 | 0.8 | 244 | - | 40 | 200 | 189 | 312 | 26 | 0.71 | 0.27 | Comparative Example |
| 8 | D | 120 | 1051 | 28 | No | 54 | 2.4 | 526 | - | 20 | 76 | 169 | 369 | 175 | 0.43 | 0.56 | Example |
| 9 | E | 137 | 1180 | 39 | No | 51 | 9.6 | 315 | 600 | 15 | 81 | 152 | 427 | 167 | 0.86 | 0.92 | Example |
| 10 | E | 130 | 1158 | 37 | No | 56 | 63.2 | 587 | - | 14 | 97 | 127 | 680 | 182 | 0.52 | 0.28 | Comparative Example |
| 11 | F | 150 | 1230 | 32 | No | 53 | 9.3 | 306 | - | 37 | 173 | 177 | 301 | 39 | 0.44 | 0.15 | Comparative Example |
| 12 | F | 200 | 1077 | 26 | No | 37 | 28.2 | 379 | - | 19 | 110 | 176 | 328 | 208 | 0.92 | 1.04 | Example |
| 13 | G | 103 | 1169 | 30 | No | 44 | 44.7 | 447 | 550 | 18 | 72 | 81 | 350 | 177 | 0.74 | 0.98 | Example |
| 14 | G | 119 | 1086 | 21 | No | 64 | 3.1 | 462 | - | 16 | 189 | 15 | 370 | 36 | 0.27 | 0.33 | Comparative Example |
| 15 | H | 144 | 1185 | 36 | No | 44 | 49.0 | 560 | 600 | 19 | 93 | 72 | 452 | 182 | 0.61 | 0.72 | Example |
| 16 | H | 124 | 1110 | 39 | No | 27 | 2.8 | 453 | - | 39 | 71 | 132 | 307 | 22 | 0.59 | 0.22 | Comparative Example |
| 17 | I | 142 | 1153 | 34 | No | 38 | 2.4 | 364 | - | 14 | 84 | 132 | 527 | 149 | 0.62 | 0.83 | Example |
| 19 | J | 170 | 1105 | 27 | No | 34 | 3.7 | 404 | - | 19 | 89 | 193 | 424 | 172 | 0.53 | 0.97 | Example |
| 20 | K | 149 | 1017 | 40 | No | 39 | 3.2 | 540 | - | 15 | 104 | 170 | 415 | 182 | 0.73 | 1.04 | Example |
| 21 | L | 127 | 1178 | 35 | No | 41 | 5.3 | 477 | - | 13 | 96 | 77 | 483 | 144 | 0.50 | 0.69 | Example |
| 22 | M | 130 | 1066 | 36 | No | 56 | 6.6 | 600 | - | 18 | 78 | 141 | 461 | 183 | 0.52 | 1.28 | Example |
| 23 | N | 140 | 1111 | 33 | No | 52 | 35.9 | 582 | 650 | 11 | 92 | 107 | 516 | 184 | 0.56 | 0.54 | Example |
| 24 | O | 126 | 1006 | 33 | No | 40 | 14.2 | 399 | - | 19 | 89 | 21 | 425 | 170 | 0.14 | 0.29 | Comparative Example |
| 25 | P | 141 | 1142 | 45 | No | 43 | 2.9 | 588 | - | 15 | 110 | 275 | 380 | 159 | 0.26 | 0.21 | Comparative Example |
| 26 | Q | 132 | 1110 | 49 | No | 51 | 8.5 | 425 | - | 12 | 94 | 164 | 492 | 142 | 0.18 | 0.17 | Comparative Example |
| 27 | R | 148 | 1146 | 40 | No | 37 | 24.6 | 557 | - | 20 | 88 | 62 | 310 | 216 | 0.68 | 0.87 | Comparative Example |
| 28 | S | 126 | 1069 | 38 | No | 37 | 14.1 | 403 | 500 | 14 | 86 | 83 | 494 | 135 | 0.26 | 0.29 | Comparative Example |
| 29 | T | 136 | 1176 | 34 | No | 56 | 6.5 | 481 | - | 18 | 83 | 114 | 520 | 184 | 0.19 | 0.27 | Comparative Example |
| 30 | U | 131 | 1112 | 44 | No | 35 | 4.4 | 211 | - | 31 | 97 | 96 | 311 | 73 | 0.47 | 0.20 | Comparative Example |
| 31 | V | 146 | 1153 | 42 | No | 44 | 4.1 | 473 | - | 14 | 79 | 108 | 372 | 219 | 0.22 | 0.13 | Comparative Example |
| 32 | W | 129 | 1130 | 37 | No | 35 | 4.9 | 535 | - | 20 | 106 | 216 | 350 | 196 | 0.23 | 0.33 | Comparative Example |
| 33 | X | 120 | 1183 | 33 | No | 44 | 21.7 | 467 | 500 | 20 | 90 | 169 | 427 | 196 | 0.11 | 0.25 | Comparative Example |
| 34 | Y | 107 | 1137 | 34 | No | 58 | 1.9 | 491 | - | 13 | 80 | 195 | 474 | 193 | 0.23 | 0.20 | Comparative Example |
| 35 | Z | 109 | 1197 | 41 | No | 63 | 7.9 | 546 | - | 12 | 88 | 190 | 386 | 175 | 0.25 | 0.28 | Comparative Example |
| 36 | AA | 101 | 1108 | 49 | No | 53 | 43.0 | 215 | 600 | 15 | 85 | 119 | 293 | 212 | 0.91 | 1.23 | Comparative Example |
| 37 | AB | 111 | 1192 | 43 | No | 54 | 6.6 | 491 | - | 13 | 100 | 91 | 495 | 197 | 0.32 | 0.12 | Comparative Example |
| 38 | AC | 141 | 1167 | 35 | No | 38 | 36.4 | 328 | - | 10 | 81 | 186 | 499 | 81 | 0.23 | 0.23 | Comparative Example |
| 39 | AD | 114 | 1116 | 37 | No | 58 | 7.3 | 530 | - | 18 | 77 | 121 | 445 | 182 | 0.29 | 0.29 | Comparative Example |
| 40 | AE | 141 | 1131 | 43 | No | 36 | 6.5 | 524 | - | 17 | 71 | 270 | 371 | 216 | 0.23 | 0.28 | Comparative Example |
| 41 | AF | 103 | 1156 | 38 | No | 64 | 30.9 | 540 | 650 | 19 | 108 | 19 | 409 | 190 | 0.16 | 0.15 | Comparative Example |
| 42 | AG | 126 | 1025 | 40 | No | 57 | 3.1 | 496 | - | 16 | 102 | 49 | 395 | 191 | 0.24 | 0.26 | Comparative Example |
| 43 | AH | 112 | 1200 | 47 | No | 35 | 4.0 | 566 | - | 14 | 94 | 97 | 511 | 37 | 0.37 | 0.19 | Comparative Example |
| 44 | AI | 143 | 1045 | 28 | No | 39 | 2.9 | 524 | - | 19 | 103 | 59 | 404 | 173 | 0.25 | 0.39 | Comparative Example |
| 45 | AJ | 128 | 1027 | 39 | No | 51 | 2.2 | 470 | - | 17 | 103 | 41 | 427 | 154 | 0.17 | 0.20 | Comparative Example |
| 46 | AK | 130 | 1176 | 27 | No | 45 | 1.9 | 461 | - | 11 | 95 | 101 | 414 | 154 | 0.25 | 0.24 | Comparative Example |
| 47 | AL | 111 | 1048 | 35 | No | 60 | 3.4 | 443 | - | 13 | 89 | 29 | 480 | 123 | 0.17 | 0.56 | Comparative Example |
| 48 | AM | 143 | 1118 | 27 | No | 55 | 1.9 | 498 | - | 18 | 105 | 147 | 487 | 205 | 0.19 | 0.29 | Comparative Example |
| 49 | AN | 126 | 1196 | 36 | No | 40 | 2.8 | 488 | 500 | 15 | 105 | 164 | 297 | 212 | 1.03 | 1.11 | Comparative Example |
| 50 | AO | 132 | 1143 | 29 | No | 43 | 4.3 | 589 | - | 15 | 77 | 130 | 389 | 149 | 0.19 | 0.24 | Comparative Example |
| 51 | AP | 107 | 1085 | 32 | No | 46 | 5.0 | 457 | - | 18 | 100 | 179 | 529 | 209 | 0.18 | 0.15 | Comparative Example |
| 52 | AQ | 135 | 1031 | 43 | No | 39 | 8.6 | 336 | - | 13 | 103 | 20 | 404 | 179 | 0.22 | 0.72 | Comparative Example |
| 53 | AR | 140 | 1196 | 38 | No | 50 | 7.2 | 553 | - | 20 | 100 | 62 | 493 | 124 | 0.22 | 0.28 | Comparative Example |
| 54 | A | 101 | 1120 | 35 | Yes | 50 | 3.4 | 376 | - | 18 | 205 | 109 | 308 | 87 | 0.54 | 0.28 | Comparative Example |
| 55 | B | 120 | 1130 | 45 | Yes | 50 | 3.2 | 401 | - | 17 | 189 | 68 | 312 | 76 | 0.61 | 0.31 | Comparative Example |
| 56 | C | 130 | 1100 | 60 | Yes | 30 | 2.7 | 421 | - | 19 | 176 | 134 | 305 | 43 | 0.49 | 0.29 | Comparative Example |
| 57 | D | 120 | 1100 | 60 | Yes | 30 | 3.3 | 399 | - | 18 | 181 | 128 | 314 | 38 | 0.71 | 0.30 | Comparative Example |

| | | | | | | | | | | | | | | | | | |
|---|---|---|---|---|---|---|---|---|---|---|---|---|---|---|---|---|---|
| Note: underlining indicates value outside scope of present disclosure | | | | | | | | | | | | | | | | | |

As can be seen from Table 2, steel plates that satisfied the conditions of the present disclosure (Examples) were produced under production conditions that fell within the scope of the present disclosure, and the base metal had values for average effective crystal grain size, maximum effective crystal grain size, and number density of composite inclusions containing sulfides containing Ca and Mn and oxides containing Al that all fell within the scope of the present disclosure. The results exhibited excellent base metal properties, with a yield stress of 325 MPa and a base metal vE-_{40 °C} of 100 J or more. Further, excellent joint CTOD properties were provided, as both the CTOD value of the CGHAZ and the CTOD value of the SC/ICHAZ boundary (δ) were 0.40 mm or more at -20 °C.

In contrast, steel plates that did not satisfy the conditions of the present disclosure (Comparative Examples) were inferior to the Example steel plates in either or both of the base metal properties and joint CTOD properties.

## Claims

1. A steel plate having a thickness exceeding 100 mm and comprising a chemical composition containing, in mass%,
C: 0.03 % to 0.13 %,
Si: 0.60 % or less,
Mn: 0.9 % to 2.7 %,
P: 0.050 % or less,
S: 0.0050 % or less,
Al: 0.002 % to 0.100 %,
Ti: 0.002 % to 0.055 %,
Nb: 0.005 % to 0.070 %,
Ca: 0.0005 % to 0.0200 %,
N: 0.0120 % or less, and
O: 0.0070 % or less,
with the balance being Fe and inevitable impurity, wherein
the chemical composition satisfies Expressions (1) to (4) below: $1.50 \leq \left[Ti\right] / \left[N\right] \leq 5.00$ $0 \leq \left\{\left[Ca\right]-\left(0.18+130\left[Ca\right]\right)\times \left[O\right]\right\} / 1.25 / \left[S\right] \leq 1.50$ 0.280 % ≤ Ceq (= [C] + [Mn]/6 + ([Cu] + [Ni])/15 + ([Cr] + [Mo] + [V])/5) ≤ 0.500 % Pcm (= [C] + [Si]/30 + ([Mn] + [Cu] + [Cr])/20 + [Ni]/60 + [Mo]/ 15 + [V]/10 + 5[B]) ≤ 0.240 %
where the square brackets in Expressions (1) to (4) indicate content in mass% of an element enclosed in the brackets and have a value of 0 when the element is not contained,
in a mid-thickness part, average effective crystal grain size is 20 µm or less and maximum effective crystal grain size is 150 µm or less, and
at a 1/2 thickness position, composite inclusions containing sulfides containing Ca and Mn and oxides containing Al and having a circle equivalent diameter of 0.1 µm or more are present at a number density of 25/mm² to 250/mm².

2. The steel plate according to claim 1, wherein the chemical composition further contains, in mass%, at least one selected from the group consisting of
Ni: 2.5 % or less,
Cu: 2.0 % or less,
Cr: 1.5 % or less,
Mo: 1.5 % or less,
V: 0.25 % or less,
W: 0.45 % or less,
B: 0.0045 % or less,
REM: 0.025 % or less and,
Mg: 0.005 % or less.

3. A method of producing a steel plate, the method comprising:
heating a material having the chemical composition defined in claim 1 or 2 to a temperature of 990 °C or more and 1210 °C or less; then rolling with an average rolling reduction per pass of 3 % or more and a cumulative rolling reduction ratio of 25 % or more when a mid-thickness temperature is T₁ °C or more as defined in Expression (5) below; rolling with a cumulative rolling reduction ratio of 30 % or more when the mid-thickness temperature is T₂ °C or less as defined in Expression (6) below; and then cooling at an average cooling rate of 1.0 °C/s to 50.0 °C/s in the mid-thickness temperature to a cooling stop temperature of 600 °C or less,
[Math. 1] ${T}_{1} = 174 log \left[sol.\left[Nb\right]\times \left(\left[C\right]+\frac{12}{14}\left[N\right]\right)\right] + 1444$
wherein sol.[Nb] is derived from Expression (7),
[Math. 2] ${T}_{2} = {T}_{1} - 75$
[Math. 3] $sol . \left[Nb\right] = exp \left[2.3\left\{2.26-\frac{6770}{{T}_{0} + 273}-log\left(\left[C\right]+\frac{12}{14}\left[N\right]\right)\right\}\right]$
and in Expressions (5) and (7), [C] and [N] represent mass% of C and N content, respectively, T₀ represents heating temperature of the material in °C, and sol.[Nb] represents Nb solute in mass%, and sol.[Nb] ≤ [Nb] where [Nb] is the total Nb content in mass% in the steel plate.

4. The method of producing a steel plate according to claim 3, wherein, after the cooling to the cooling stop temperature, a tempering treatment is performed at a temperature of 700 °C or less.
